

## UNITED STATES PATENT OFFICE.

FREDERICK W. ROHRS, OF BALTIMORE, MARYLAND.

## MOTOR FUEL.

No Drawing.

Application filed December 17, 1921. Serial No. 523,193.

*To all whom it may concern:*

Be it known that FREDERICK W. ROHRS, a citizen of the United States, residing at Baltimore, in the county of Baltimore City and State of Maryland, has invented new and useful Improvements in Motor Fuel, of which the following is a specification.

This invention, which is a continuation in part of applicant's co-pending application, 10 S. N. 447,248, Patent No. 1,425,136, Aug. 8, 1922, relates to liquid fuel for use in internal combustion engines, and has for its object to provide a fuel, which, due to possessing a higher specific gravity than the common 15 commercial form of gasoline, is heavier, and gives a slower combustion, and will permit of a higher spark advance to the engine than heretofore possible with the ordinary type of fuel now on the market.

20 By utilizing a heavy fuel comprising the ingredients in the proportions herein set forth, it is obvious that a considerable saving will be effected in the consumption of the fuel, as the same will not be drawn off 25 and burned as wastefully from the jet of the carburetor as the lighter and more volatile fuels.

The motor fuel is composed of the petroleum distillate products, gasoline and kerosene, which are admixed with acetone and benzol in substantially the proportions below set forth.

35 A motor fuel compounded in accordance with my invention will greatly increase the mileage per gallon of the fuel, and at the same time improve the efficiency and increase the durability of the motor, as it will not corrode or have any other detrimental effect upon the engine parts.

40 Furthermore, the fuel has the effect of keeping the carbon in the cylinders in suspension, preventing its hardening on the metal surfaces, and thus permitting the said free carbon to be expelled through the exhaust.

45 At temperatures ranging between 0° F. and 10° F., the following ingredients in the percentages below set forth have been found to give very advantageous results:

50 Acetone, approximately 3%.

Benzol, approximately 9%.

Petroleum distillate, approximately 88%.

The percentage of petroleum distillate being composed of approximately 85% gasoline and 3% kerosene.

In order that a heavy blended fuel may be obtained at various degrees of temperature, it has been found desirable to vary the increases of benzol for changes in atmospheric temperatures, between 10° F. to 100° F., from 60 approximately 7% to 80% without any variation being made in any of the other ingredients.

At a temperature of 70° F. the fuel when mixed with the following ingredients has 65 proved highly satisfactory:

Acetone, approximately 1%.

Petroleum distillate, approximately 49%.

Benzol, approximately 50%.

In the above formula, the composition 70 percentage of petroleum distillate is composed of approximately 1% kerosene, and 48% gasoline.

At a temperature of 100° F., the ingredients in the following percentages have been 75 found to give the best results:

Acetone, approximately 1%.

Benzol, approximately 79%.

Petroleum distillate, approximately 20%.

The petroleum distillate in the above composition being composed of approximately 80 29% gasoline and 1% kerosene.

The varying of the quantity of benzol used has been found desirable, since benzol at a very low temperature has a tendency to 85 change from the fluid to the solid state, and this congealing naturally tends to impair the efficiency of the fuel, if not proportionately lessened as the temperature decreases. Conversely, the benzol must be proportionately increased as the temperature rises. By thus varying the quantity of the benzol as the temperature changes, a heavy and slowly burning fuel is obtained, which will permit of a higher spark advance, together 90 with a resultant increase in the compression of the cylinders, and a reduction in the consumption of the fuel.

The acetone, due to its mobility, tends to 100 produce better vaporization of the fuel, thus causing the engine to start much easier. It also counteracts the heating effect of the benzol, and assists materially in keeping the temperature of the engine at a proper point.

The kerosene tends greatly to facilitate 105 the mixing and blending of the acetone with the gasoline, and also prevents the too rapid vaporization of the acetone. Another important advantage residing in the use of kerosene is, that it acts, in combination with 110

2  
the acetone, as a solvent of the carbon developed in the cylinders, and causes the carbon to remain continuously in suspension so that the free carbon is readily expelled with 5 the exhaust gases, which results in the elimination of the carbon deposits in the cylinders.

By my invention, I am able to materially cut down the use of gasoline, and yet secure 10 a fuel which is high in power and in mileage per fuel unit, and which will have a lower vaporization point than commercial gasoline, so that losses from excessive and rapid vaporization are materially reduced.

15 While I have above set forth the proportions of the ingredients which I at present prefer to employ, I do not wish to be limited to the exact proportions herein given, as the same may be varied to a considerable 20 extent and still be within the range of my invention.

I claim:

1. A motor fuel comprising from 1 to 3 parts of acetone, 25 to 35 parts of petroleum 25 distillate, and 50 to 80 parts benzol, said parts of benzol varying from the minimum

to the maximum above set forth in direct variation to the increase in temperature.

2. A motor fuel comprising from 1 to 3 parts acetone, 1 to 3 parts kerosene, 25 to 30 30 parts gasoline, and 50 to 80 parts benzol, said parts of benzol increasing from the minimum to the maximum above set forth in direct variation to the increase in temperature.

3. A motor fuel comprising approximately 1% acetone, 1% kerosene, 79% benzol, and 19% gasoline.

4. A motor fuel comprising approximately 1% acetone, 79% benzol, and 20% 40 petroleum distillate.

5. A motor fuel comprising from 1 to 3 parts acetone, 7 to 80 parts benzol, and 10 to 25 parts petroleum distillate, said parts of benzol increasing from the minimum to 45 the maximum above set forth in direct variation to the increase in the temperature from 10° F. to 100° F.

In testimony whereof I have hereunto set my hand.

FREDERICK W. ROHRS.